

Aug. 22, 1944.

A. E. LUNDBYE

2,356,329

METHOD FOR THE SEPARATION AND RECLAMATION OF  
COPPER FROM PRINTING PLATES AND THE LIKE  
Filed May 23, 1942



Inventor

Axel E. Lundbye

By

Barney Cook.

Attorney

## UNITED STATES PATENT OFFICE

2,356,329

## METHOD FOR THE SEPARATION AND RECLAMATION OF COPPER FROM PRINTING PLATES AND THE LIKE

Axel E. Lundbye, Springfield, Ohio, assignor to The Crowell-Collier Publishing Company, Springfield, Ohio, a corporation of Delaware

Application May 23, 1942; Serial No. 444,228

7 Claims. (Cl. 75—63)

My invention relates to new and useful improvements in a method for the separation and reclamation of metals and alloys that make up printing plates and printing cylinders and other articles of a like nature on which copper and nickel may have been deposited.

The present application deals more particularly with the recovery of the copper, as this metal is especially valuable and scarce at this time.

The separation and reclamation of the nickel and the backing metals from the plates will be mentioned, but the process for the recovery of the nickel forms the subject matter of my application Serial No. 447,582, filed June 18, 1942.

As is well known to those skilled in the art, the printing cylinders or plates of the printing presses are composed of a base electrotype metal consisting generally of an alloy of tin, lead and antimony, then a sheet of tin foil for tinning purposes, after which there is electrolytically deposited a layer of copper, over which there is deposited a layer of nickel for the sake of hardness.

After these cylinders or printing plates have been used, they have generally been discarded or stored away, and although various means have been tried for the separation and reclamation especially of the copper, still the processes have been complicated, and the time taken to reclaim the copper covered a relatively long period, thus making the recovery not practical from a commercial standpoint.

One of the objects of the present invention, therefore, is to provide a method for the recovery of the base metal and especially for separating the copper from the backing material, and also the recovery of the nickel, so that this copper can again be made into anodes and then redeposited on new printing plates and the base metal and the nickel also recovered for re-use.

Another one of the objects of the present invention is to provide a method for the separation and reclamation of the copper which will take but a relatively short time and thus keep down the cost of the said reclamation process.

Still another object of the invention is to provide a method especially for the recovery of the copper in the used printing press plates, which method will effectively separate the copper from the other metals or alloys making up the composite plate, so that the copper reclaimed will be in as good a condition as it was when first used.

Still another object of the invention is to re-

cover the copper from the printing plates which consists in removing the nickel by an electrolytic process; removing the base by heat; subjecting the copper shell also to heat; suddenly cooling; then a knurling action to break up the scale; and a mechanical as well as a chemical cleansing operation so that the copper can be quickly and readily again used for anodes for the depositing of the copper on new printing plates and cylinders.

10 With these and other objects in view, the invention consists in certain new and novel steps for carrying out the method shortly to be outlined.

15 Referring to the drawing showing a preferred embodiment of my invention,

Fig. 1 is a small fragmentary section of a printing cylinder or plate after it has been flattened and is ready to be treated, the tin foil being enlarged for the sake of clearness of illustration;

20 Fig. 2 is similar to Fig. 1 but showing the nickel as having been removed;

Fig. 3 is a view similar to Fig. 2 and shows the copper shell remaining with its tin foil now in the uppermost position;

25 Fig. 4 is a diagrammatic view of conveyor rollers, pressure rollers, cleansing bath and means for heating the copper shell or plate on its trip to the storage station; and

30 Fig. 5 is a fragmentary view showing how the reclaimed copper shell will appear when completed.

35 As heretofore mentioned, in the method to be outlined I not only recover the copper and the nickel, but also the base material; but the recovery of these is incidental to the recovery of the copper and the recovery of the nickel forms the subject matter of my application Serial No. 447,582, filed June 18, 1942.

40 As heretofore mentioned, the printing plates as used in the large flat presses and cylindrical printing presses consist of a backing metal, which is an alloy of tin, lead and antimony, and designated by the word "Base" in the drawing.

45 In the several views I have shown the plate as being flat, rather than arcuate, but, of course, in the recovery of the metal by my method, when the plates are of cylindrical form, the cylinders are flattened, as may be seen in the several views.

50 A sheet of tin foil 2 is shown, which I have exaggerated in the several views for the sake of clearness, which tin foil is placed on the rear face of the copper which acts as a tinning agent when the base metal 3 is cast thereon.

It might be mentioned that in the formation of printing plates there is a wax or lead mold made from an original copper etching and this lead or wax mold is then plated in a nickel electroplating tank with a nickel deposit of from .001 to .0015 of an inch. The mold with the nickel thereon is then subjected to a copper plating where from .006 to .0012 of copper is plated on back of the nickel. Then the mold with its covering of nickel and copper is removed from the tank and the lead mold stripped away. The plate, now of copper and nickel, is cut down to size of the printing plate and placed in a casting machine, copper side up, and at this stage the tin foil is placed on the face of the copper. Then the backing metal that is the lead, tin and antimony is cast on the copper, the tin foil acting as a tinning medium.

It has been the general practice to store away these used plates or cylinders, and a number of processes have been devised for separating and reclaiming the metals, but these methods have not come into practical use due to the heretofore relative cheapness of the metals and their plentifullness, and further, due to the expense of the reclaiming process and the length of time that it took.

As heretofore mentioned, with the method and apparatus hereinafter mentioned, I can fully recover the various metals so that they may again be used in the making up of the new printing cylinders.

Taking a plate as shown in Fig. 1, the ink (not shown) is removed from the nickel type surface by scrubbing with a brush using kerosene or any other suitable solvent. This scrubbing may take place before the plate is straightened out or afterwards. They are then cleaned with a hot, soapy water.

After the ink has thus been removed, the plate is suspended from the anode bar of an electroplating tank (not shown).

The proper solution and sufficient density of current is used to quickly strip the metal from the outer or copper surface.

I have not shown the tank for the electrolytic stripping solution for the nickel and it might be mentioned that the solution will contain, in the proper portions, muriatic acid and boric acid in aqueous solution. The boric acid acts as a suitable buffer medium, and it is possible to strip the nickel from the plate in from three to four minutes.

During the stripping action the plates should be supported by their respective hangers, the plates being secured by one corner, and after the nickel has been removed, the corners should be sheared off, as the nickel still remains on these corners, and these shearings may then be placed in the tank and the nickel removed.

Of course, the electrolytic stripping has to be watched carefully to obtain the desired results.

After the nickel has been removed from the plate, the plate is removed and thoroughly scrubbed in running water and set aside to dry for the next step.

It might be mentioned here that what little copper has gone into the electrolyte bath may be precipitated and recovered, but the present invention relates to the main body of copper that has not been affected by the electrolytic bath.

After the printing plates have been treated as heretofore mentioned, they are now composed of a base of an alloy of lead, tin and antimony, a thin film of tin and a layer of copper.

I next take the plates which are now in the form shown in Fig. 2 and coat the upper or copper surface with a thin coating of whiting such as calcium oxide or its equivalent. After the whiting has been carefully applied, the plates are then placed in a melting pot (not shown) where the temperature is accurately controlled.

The temperature is held as close to the lower range of the melting point of the base metals as possible, as it is not desired to add more heat than is absolutely necessary to make the metal flow easily and it is desirable to keep the oxidation of the antimony and tin to the very minimum.

Before the base metal is formed into pigs it is treated with carbon and the pot is thoroughly cleaned by means of a starch compound which is also converted into carbon, and the metal agitated so that the impurities will go to the top of the pot, while the base metal is poured from the bottom of the pot.

A chemical analysis of the reclaimed base metal can be made at regular intervals to maintain the proper ratio of tin, lead and antimony. Of course, the copper plates will be at the top of the molten metal.

The whiting that was applied to the face of the copper prevents the base metal from adhering to this surface during the melting of the base metal.

The copper plate or shell appears as now shown in Fig. 3 (here again the tin foil being exaggerated for the sake of clearness of illustration) and I then place this copper shell on the conveyor rollers 6 as seen in Fig. 4.

These copper shells or plates now have a thin coating of the backing metal that adheres very tightly due to the tinning operation in the making up of the composite plate.

Of course, the tin foil has lost its original form, but it mixes with a part of the base metal and heretofore has been extremely hard to remove. However, by placing the plate on the roller 6 as heretofore mentioned, with the tinning on the upper surface, and by heating the copper shells to a bright red heat, and exposing the tinned surface—that is, the upper surface, to the air during the heating, I can oxidize the remaining tin and backing metal and turn it into a hard, brittle scale in the course of from fifteen seconds to two minutes.

To provide the heat, there is shown a plurality of gas jets 7 positioned between the rollers 6 playing directly on the copper or under surface of the plate.

To further assist in loosening the oxidized scale from the copper shell, the shell is advanced beneath a cold spray, as shown at 8, and this sudden cooling of the hot plate materially assists in also loosening and removing the unwanted oxidized scale.

The plate then continues on its travel and passes between the first two knurling rollers 9, which tend to bend or corrugate the copper plate, as may be seen in Fig. 5.

After passing through the first two knurling rollers, the plate then passes through the second pair of knurling or crimping rollers 9 which are arranged to bend or undulate the metal in an opposite direction. In other words, the small areas are first bent upwardly by the one set of rollers, and then downwardly by the second, and this corrugating or bending action further pulverizes and loosens the scale of oxidized metal, thus leaving the copper relatively clean.

To further assist in the cleaning action, I place a revolving wire brush 10 just beyond the knurling rollers 9 to remove any of the flakes that are still on the plate, and after the plate passes beneath this wire brush, the plate is then passed into a tank 11 in which there may be a muriatic acid bath (HCl) to thoroughly cleanse the plate from the oxidized backing material, and the plate is again scrubbed by a second revolving wire brush 12 after the plate has moved on the conveying roller 6 out of the tank. The whiting is removed from the plate by the above-described cleaning operations.

Finally the plate moves under a spray jet where it is again washed to remove the muriatic acid and then drops to a storage bin 13.

The plates are then dried and may then be remelted and cast to be again used as anodes for depositing the copper on the base metal, as heretofore mentioned.

It might be mentioned that one of the critical steps of the method is the applying of the proper heat in a uniform manner to the copper plate, in order to thoroughly oxidize the film of backing metal. If this film is not thoroughly oxidized, it will not separate from the copper during the crimping process of the roller.

However, with the proper application of heat to the copper, the lead, antimony and tin can be properly oxidized in from fifteen seconds to two minutes, as heretofore mentioned.

From the foregoing it will be seen that I have devised a method wherein all the metals that make up the printing plates or other similar articles can be saved and reclaimed, the reclamation of the copper being the important metal at this time.

It will be seen that the entire method from the scrubbing and flattening of the plates until the time they have passed through the electrolytic bath, melting pot and apparatus mentioned, consumes but a relatively short time, so that the method is not an expensive one but, on the other hand, relatively fast and relatively inexpensive.

It will be understood that the heating and cooling operations, and the electrolytic action must be watched and regulated, but I have found the method in actual practice to give excellent results and quickly and readily separates the various metals from each other, and especially separates all of the tinning and base metal from the copper plate, so that the copper can be remelted, cast and re-used as anodes with the same effect as if the copper were virgin, rather than reclaimed.

It will also be seen that the apparatus may be built at a low cost and occupies but a relatively small floor space.

Finally, it will be understood that by utilizing a conveyor system for the plates as diagrammatically illustrated, in which there is a receiving station, a cooling station, a knurling station, a tank and a discharge station, the apparatus can be watched by a minimum number of workers or operators to thus keep down the cost of the reclamation. It will, of course, be understood that rather than having a storage bin as mentioned, a portable truck or other means might be located under the discharge station so that the plates after being treated may be rapidly removed for recasting.

Having thus described my invention, what I claim as new and desire to secure by Letters Patent is:

1. The method of recovering copper from

printing plates made up of a base metal with a coating of copper and nickel thereon, said base metal having a lower melting point than copper, which consists in electrolytically stripping off the nickel; coating the stripped surface with a whiting; melting off the base metal which leaves but a thin coating of the same on one surface of the plate; oxidizing the thin coating by heating and rapidly cooling the plate to change the coating to a scale; distorting the surfaces of the plate in a plurality of minute areas to thus crack and loosen the scale; and removing the loosened scale from said plate.

2. The method of recovering the copper from printing plates made up of a base metal containing an alloy of lead, antimony and tin, and on which has been deposited a layer of copper and nickel, which consists in electrolytically stripping off the nickel; coating the stripped surface with a whiting; subjecting the plate to a direct heat of sufficient temperature to melt the base metal and leave but a thin coating thereof on the one surface of the plate; subjecting the non-coated surface to heat from fifteen seconds to two minutes and rapidly cooling the plate by spraying water thereon to thus oxidize the coating; subjecting the plates to rollers to bend the surfaces into a plurality of hills and valleys and then to further rollers to change the hills into valleys and vice versa to thus thoroughly crack and loosen the oxidized scale from the copper surface, and mechanically and chemically remove the loosened scale from said plate.

3. The method of separation and reclamation of copper from printing plates made up of a base metal comprising lead, tin and antimony, a layer of nickel, and a layer of copper between the base metal and nickel layer, which comprises thoroughly cleansing the plate; electrolytically stripping the nickel from the surface of the copper layer; covering the stripped surface with whiting and placing the plate in a melting pot and melting off the base metal for future recasting; heating the copper plate by directing a hot flame against the stripped surface to oxidize any film of base metal remaining on the other surface of the copper plate, subjecting the plate to a cold spray to chill the plate and make brittle the oxidized film; crimping the plate to loosen the oxidized metal film; subjecting the plate to a cleansing brush and then to a cleansing acid bath; and finally washing the plates with water to remove the acid.

4. The method of recovering copper from printing plates made up of a base metal with a coating of copper and nickel thereon, said base metal having a lower melting point than copper, which consists in electrolytically stripping off the nickel; applying a protective coating to the stripped surface, melting off the base metal which leaves but a thin coating of the same on one surface of the plate, oxidizing the thin coating by heating and rapidly cooling the plate to change the coating to a scale; distorting the surfaces of the plate in a plurality of minute areas to thus crack and loosen the scale, and removing the loosened scale from said plate.

5. The method of separation and reclamation of copper from printing plates made up of a base metal comprising lead, tin and antimony, a layer of nickel and a layer of copper between the base metal and nickel layer, which comprises thoroughly cleansing the plate, electrolytically stripping the nickel from the surface of the copper layer, covering the stripped surface with

whiting and placing the plate in a melting pot and melting off the base metal for future recasting, heating the copper plate by directing a hot flame against the stripper surface to oxidize any film of base metal remaining on the other surface of the copper plate, subjecting the plate to a cold spray to chill the plate and make brittle the oxidized film, crimping the plate to loosen the oxidized film, and cleaning the oxidized metal film from the crimped plate.

6. The method of separating and reclaiming copper from printing plates made up of a base metal, comprising lead, tin and antimony, together with successive layers of tin, copper and nickel superimposed on said base metal, which consists in thoroughly cleansing the plate, electrolytically stripping the nickel off the surface of the copper layer, covering the stripped surface with a chalk, melting off the base metal, the chalk preventing the aforementioned metal from tinning the stripped surface of the copper plate, heating the copper plate by directing a hot flame on said stripped surface to oxidize the lead, tin

and antimony which remains on the other surface of the copper plate, then quickly subjecting the plate while still hot to a cold water spray to quickly chill the plate and make brittle the remaining oxidized film, crimping the plate to distort and undulate the surfaces of the plate to thus loosen the oxidized metal film on the upper surface of the copper plate, brushing the plate to remove the scaly film, cleaning the brushed plate with acid, and finally washing the plate to remove the remains of the acid bath.

7. In a method of recovering copper from a copper plate having one relatively clean surface and a coating of a metal on the other surface thereof that oxidizes at a temperature lower than the melting point of copper, oxidizing said coating by directing a flame against said clean surface of said plate, distorting said plate in a plurality of small areas to crack and loosen the oxidized coating, and removing the loosened coating.

AXEL E. LUNDBYE.

CERTIFICATE OF CORRECTION.

Patent No. 2,356,329.

August 22, 1944.

AXEL E. LUNDBYE.

It is hereby certified that error appears in the printed specification of the above numbered patent requiring correction as follows: Page 4, first column, line 4, claim 5, for the word "stripper" read --stripped--; and that the said Letters Patent should be read with this correction therein that the same may conform to the record of the case in the Patent Office.

Signed and sealed this 3rd day of October, A. D. 1944.

Leslie Frazer

(Seal)

Acting Commissioner of Patents.